

[72] Inventors **Harald Huckstadt**  
**Cologne, Stammheim;**  
**Erwin Ranz, Leverkusen; Herbert**  
**Grabhofer, Cologne, Flittard, all of**  
**Germany**  
[21] Appl. No. **852,073**  
[22] Filed **Aug. 21, 1969**  
[45] Patented **Oct. 26, 1971**  
[73] Assignee **AGFA-Gevaert Aktiengesellschaft**  
**Leverkusen, Germany**  
[32] Priority **Sept. 6, 1968**  
[33] **Germany**  
[31] **P 17 97 263.3**

[54] **SILVER HALIDE EMULSIONS WHICH CONTAIN COLOR COUPLERS**  
10 Claims, No Drawings  
[52] **U.S. Cl.** ..... **96/55,**  
96/100, 96/107, 96/114  
[51] **Int. Cl.** ..... **G03c 7/00,**  
G03c 1/28

[50] **Field of Search** ..... **96/55, 100,**  
**107**

[56] **References Cited**  
**UNITED STATES PATENTS**  
2,944,900 7/1960 Carroll et al. .... 96/100  
3,370,048 2/1968 Reynolds. .... 96/107  
3,471,296 10/1969 Huckstadt et al. .... 96/107

*Primary Examiner*—J. Travis Brown  
*Attorney*—Connolly and Hutz

**ABSTRACT:** The sensitivity of a light-sensitive photographic material containing in the silver halide emulsion layer a color coupler capable of forming a dye upon reaction with the oxidation product of a color-forming developer is increased by addition of a water-soluble quaternisation product of an  $\alpha,\omega$ -bis-(thiomorpholinyl)-alkane with a bifunctional polyalkylene oxide.

## SILVER HALIDE EMULSIONS WHICH CONTAIN COLOR COUPLERS

The invention relates to a process for increasing the sensitivity of photographic silver halide emulsions which contain color couplers as well as to color photographic silver halide emulsions with improved sensitivity.

It is known that the sensitivity of photographic silver halide emulsions can be increased by the addition of so-called development accelerators or chemical sensitizers. Polyalkylene oxides and their derivatives have, inter alia, been described for this purpose. It is also known that in addition to simple polyalkylene oxides of different chain lengths, polyalkylene oxides with onium substituents may be used as chemical sensitizers.

Most of these compounds, however, have the disadvantage that in addition to increasing the sensitivity, they increase the fog of the emulsion. In many cases, these two factors are very adversely related to each other. This applies particularly to silver halide emulsions which contain color couplers, such emulsions being particularly liable to fogging.

Furthermore, it is known to use water-soluble quaternization products of tertiary polyamines with bifunctional polyalkylene oxide derivatives which contain open chain dialkylamines as chemical sensitizers for silver halide emulsions. The effectiveness of these compounds in color emulsions, however, is unsatisfactory.

It is among the object of the invention to provide chemical sensitizers for silver halide emulsions which contain color couplers which, while greatly increasing the sensitivity without concomitant increase of fogging.

We now have found that water-soluble quaternization products of  $\alpha$ ,  $\omega$ -bis-(thiomorpholinyl)-alkanes with bifunctional polyalkylene oxide derivatives are excellently suitable for use as development accelerators or chemical sensitizers for silver halide emulsions which contain color couplers.

The compounds have the following general formula:



IV



V



VI



wherein represents

$a = 2$  to  $6$ ,

$n = 3$  to  $300$ ,

$y = 2$  to  $10$ , preferably  $2$  to  $5$ ,

$x = \text{any anion, e.g. halide, perchlorate, benzene sulfonate or the like.}$

The anion may be chosen according to the requirements of the process used for the preparation since its chemical nature for the sensitizing effect is of minor importance.

Particular utility is exhibited by the following compounds:

I



20



30

III



40

M=51000

4,1

V



4,4

VI



3,1

VII



VIII



The molecular weights given must be regarded as average values owing to the comparative inaccuracy of the methods of determination.

The substances according to the invention are prepared by quaternizing a bis-(thiomorpholinyl)-alkane, for example with the bis-tosylate of a polyalkylene oxide of desired chain length. The method of preparation will be described in the following with reference to compound II:

#### STAGE I

Fifty-one g. of thiomorpholine and 20 g. of sodium hydroxide are dissolved in 75 ml. of water. 47 of ethylene bromide are added dropwise with stirring at boiling point and the reaction mixture is refluxed for several hours. Thereafter it is concentrated by evaporation. The product, bis-(thiomorpholinyl)-ethane-(1,2), separates in the form of colorless crystals which melt at 97° to 98° C. Yield 36g.

#### STAGE II

Thirty-three g. of a polyethylene bistosylate which has an average molecular weight of about 1350 and 6.9 g. of the above bis-(thiomorpholinyl)-ethane-(1,2) are heated under reflux for 3 hours with 50 ml. of butanol. After evaporation of the solvent, compound II is obtained as a brownish waxy substance. Yield 38 g.

The substances according to the invention may be added to the photographic emulsion at any stage of its preparation before, during or after chemical ripening. They may also be added to the casting solution immediately before casting. The quantity added depends on the desired effect and can easily be determined by the expert by the usual tests. Quantities of 0.1 to 10 g. per mol of silver halide will normally be sufficient.

The substances according to the invention may be used in any silver halide emulsions which contain color couplers. Suitable silver halides are silver chloride, silver bromide or mixtures thereof, if desired, containing a small amount of silver iodide of up to 10 mols percent. The silver halides may be dispersed in the usual hydrophilic compounds, for example in carboxymethyl cellulose polyvinyl alcohol, polyvinyl pyrrolidone, alginic acid and its salts, esters or amides or, preferably, in gelatine.

The emulsions can also be optically sensitized with cyanine

25 dyes such as basic or acid carbocyanines, cyanine dyes of the betaine type, rhodacyanine or merocyanine dyes, styryl or oxonol dyes. Suitable sensitizers are described by F. M. Hamer "The Cyanine Dyes and related Compounds." Interscience Publishers, (1964).

30 The emulsions may also contain chemical sensitizers, e.g. reducing agents such as stannous salts, polyamines such as diethyltriamine or aminomethane sulfonic acids or derivatives thereof such as described in Belgian patent specification No.

35 547,323 or sulfur compounds as described in U.S. Pat. No 1,574,944, for example allyl thiocyanate, allylthiourea, sodiumsulfate and the like. Suitable chemical sensitizers are also salts of noble metals such as ruthenium, rhodium, palladium, iridium, platinum or gold, as described in the article by R.

40 Koslowsky, Z. wiss.phot. 46, 65-72 (1959). Further suitable for chemical sensitization are polyalkylene oxides, especially polyethylene oxide having an average molecular weight of 1,000 to 20,000 and derivatives thereof, such as condensation products of alkylene oxides with aliphatic alcohols, glycols

45 cyclic dehydration products of hexitols, alkyl substituted phenols, aliphatic carboxylic acids, aliphatic amines, diamines or amides. The said condensation products have preferably a molecular weight of above 1,000. It is also possible to apply combinations of several chemical sensitizers.

50 Particular suitable for the emulsion of the present invention are chemical sensitizers of the thiomorpholine series such as described in French Pat. No. 1,506,230.

55 The emulsions according to the invention may additionally contain the usual stabilizers, e.g. homopolar or salt-type compounds of mercury with aromatic or heterocyclic rings, such as mercaptotriazoles, simple mercury salts, sulfonium mercury double salts, and other mercury compounds. Other stabilizers

60 which may be used include azaindenes, especially tetraazaindenes or pentaazaindenes, in particular those substituted with hydroxyl or amino groups. Compounds of this type have been described in the article by Birr, Z. wiss.phot. 47, 2-58 (1952). Other suitable stabilizers include heterocyclic mercapto com-

65 pounds, e.g. 1-phenyl-5-mercapto-tetrazole, quaternary benzthiazole derivatives and benztriazoles.

The emulsions may be hardened in the usual manner, for example, with formaldehyde or halogen-substituted aldehydes that contain a carboxyl group, e.g. mucobromic acid, diketones, methanesulfonic acid esters and dialdehydes.

70 The substances described may also be added to the developer, although they are less effective when used in this way. Amounts of 1 to 20 g. per 1. of the aqueous developing composition have proved sufficient.

## EXAMPLE 1

A mixed emulsion composed of 90 percent of a silver iodobromide gelatine emulsion and 10 percent of a silver iodochlorobromide gelatine emulsion, which mixed emulsion has been ripened to optimum sensitivity in known manner with gold compounds and sulfur compounds is sensitized by the addition of 45 mg. of the following sensitizing dye per kg. of emulsion:



In addition, the following ingredients are added per kg. of emulsion:

- 15 g. of 1-(3'-sulfo-4'-phenoxy)-phenyl-3-heptadecyl-pyrazolone as magenta coupler,  
 250 mg. of 1,3,3a,7-tetraaza-4-hydroxy-6-methylindene as stabilizer,  
 20 ml. of a 5 percent aqueous solution of saponin as wetting agent,  
 2.5 ml. of a 30 percent aqueous solution of formaldehyde as hardener.

The emulsion is divided into 10 parts and the following substances per kg. of emulsion are added to the individual parts:

- Sample A: Comparison sample without additive.  
 Sample B: 300 mg. of Substance I.  
 Sample C: 300 mg. of Substance III.  
 Sample D: 1 g. of Substance IV.  
 Sample E: 300 mg. of Substance V.  
 Sample F: 300 mg. of Substance VI.  
 Sample G: 300 mg. of Substance VII.  
 Sample H: 300 mg. of Substance VII of British Pat. specification No. 1,145,186 of the following formula:



Sample I: 300 mg. of Substance No. XIII of British Pat. specification No. 1,145,186 of the following formula:



Sample K: 1.2 g. of Substance No. XIII of the British patent specification referred to above.

The table I given below clearly shows the superior effect of the sensitizing compounds of the present invention.

The samples are applied onto a cellulose acetate support and dried. They are then exposed behind a step wedge and processed as follows:

|                   |            |
|-------------------|------------|
| Color development | 7 minutes  |
| Short stop bath   | 5 minutes  |
| washing           | 5 minutes  |
| Bleaching bath    | 5 minutes  |
| Washing           | 5 minutes  |
| Fixing bath       | 5 minutes  |
| Washing           | 10 minutes |

10 The color developer has the following composition:

|                                        |         |
|----------------------------------------|---------|
| N,N-Diethyl-p-phenylenediamine sulfate | 2.75 g. |
| Hydroxylamine sulfate                  | 1.2 g.  |
| Sodium sulfite anhydrous               | 2.0 g.  |
| Sodium hexametaphosphate               | 2.0 g.  |
| Potassium carbonate anhydrous          | 75.0 g. |
| Potassium bromide                      | 2.0 g.  |
| Make up to 1 liter with water.         |         |

20 The other treatment baths had the following composition:

|                  |                        |         |
|------------------|------------------------|---------|
| short stop bath: | sodium acetate         | 30.0 g. |
|                  | Glacial acetic acid    | 6.0 g.  |
|                  | Make up with water to  | 1 l.    |
| Bleaching bath:  | Potassium ferricyanide | 100 g.  |
|                  | Potassium bromide      | 20 g.   |
|                  | Disodium phosphate     | 10 g.   |
|                  | Glacial acetic acid    | 4 g.    |
|                  | Make up with water to  | 1 l.    |
| 30 Fixing bath:  | Sodium thiosulfate     | 200 g.  |
|                  | Make up with water to  | 1 l.    |

35 The color density of the magenta layers was determined with a "Macbeth Quanta Log, Model TD 102" densitometer, a green color filter being interposed in the path of the beam of measuring light.

TABLE I

| Sample | Sensitivity | $\gamma$ | Fog   |
|--------|-------------|----------|-------|
| A      | Standard    | 0.67     | 0.15  |
| B      | +5.2°       | 0.66     | 0.028 |
| C      | +3.9°       | 0.67     | 0.24  |
| D      | +4.2°       | 0.67     | 0.23  |
| E      | +3.5°       | 0.67     | 0.26  |
| F      | +3.7°       | 0.66     | 0.23  |
| G      | +4.1°       | 0.69     | 0.24  |
| H      | +1.7°       | 0.67     | 0.26  |
| I      | +1.8°       | 0.68     | 0.27  |
| K      | +2.1°       | 0.70     | 0.30  |

55 3° denote a difference of one shutter stop.

## EXAMPLE 2

60 To the emulsion described in example 1 are added an optical sensitizer for the red region of the spectrum (40 mg./kg.) of the formula:



and the cyan coupler of the following formula:



Subsequent working up is carried out as given in Example 1.

TABLE 3

| Sample | Sensitivity | $\gamma$ | Fogging |
|--------|-------------|----------|---------|
| A      | Standard    | 0.77     | 0.13    |
| B      | +3.7°       | 0.60     | 0.20    |
| C      | +3.2°       | 0.61     | 0.20    |
| D      | +3.1°       | 0.67     | 0.18    |
| E      | +2.7°       | 0.66     | 0.20    |
| F      | +2.8°       | 0.66     | 0.20    |
| G      | +3.0°       | 0.64     | 0.23    |
| H      | +3.2°       | 0.64     | 0.20    |
| I      | +1.7°       | 0.66     | 0.23    |
| K      | +1.5°       | 0.62     | 0.21    |
| L      | +1.9°       | 0.66     | 0.29    |

3° denote a difference of one shutter stop.

20

## EXAMPLE 4

A silver iodobromide gelatine emulsion containing 0.25 mol. of silver bromide and 0.016 mol. of silver iodide per kg. is used as basis for a multilayered color photographic negative material. The individual layers are optically sensitized as described in examples 1 and 2 (the blue sensitive top layer emulsion in this case does not contain an optical sensitizer) and the following color couplers are added:

25 1 kg. of the red sensitive emulsion of example 2 containing 20 g. of the cyan coupler 1-hydroxy-N-octadecyl-2-naphthamide and the casting additives given in example 1 is applied onto a cellulose triacetate support.

30 On that layer is coated the green sensitive emulsion of example 1 which contains per kg. 16 g. of magenta coupler 1-(4'-phenoxy-3'-sulfo)-3-heptadecyl-pyrazolone-5 and the other casting additives given in example 1. A yellow filter layer of colloidal silver is cast on the green-sensitive layer. The top layer consists of the nonsensitized emulsion of example 3 which contains 20 g. of yellow coupler 3-stearylaminobenzoyl-3',5'-dicarboxyacetanilide and the other additives of example 1.

35 The above multilayer material is used as comparison sample (Sample A).

40 A second multilayer material (Sample B) was made in the same way but in addition contains 500 mg. of compound II per kg. of emulsion in each emulsion layer.

45 Samples A and B are exposed to white light behind a grey step wedge and developed for 8 minutes in a developer of the following composition:

N,N-Diethyl-p-phenylenediamin sulfate—2.75 g.

Hydroxylamine sulfate—1.2 g.

Sodium carbonate anhydrous—2.0 g.

Sodium hexametaphosphate—2.0 g.

Potassium carbonate anhydrous—75.0 g.

Potassium bromide—2.5 g.

Water up to—1,000 ml.

50 60 The samples are furthermore processed as described in examples 1 to 3.

The results of the sensitometric tests are shown in table 4.

TABLE 4

| Sample    | Sensitivity | $\gamma$ | Fog  |
|-----------|-------------|----------|------|
| A yellow  | Standard    | 0.73     | 0.28 |
| B yellow  | +2°         | 0.75     | 0.30 |
| A magenta | Standard    | 0.68     | 0.25 |
| B magenta | +2°         | 0.70     | 0.27 |
| A cyan    | Standard    | 0.75     | 0.18 |
| B cyan    | +2°         | 0.78     | 0.20 |

An increase by 3° corresponds to a sensitivity increase of one shutter stop.

75

3° denote a difference of one shutter stop.

## EXAMPLE 3

To the emulsion described in example 1 are added 15 g. of the yellow coupler of the following formula:



without the addition of an optical sensitizer.

The other additives are the same as in example 1. The emulsion is divided into 11 parts and the following substances are given per kg. of emulsion to the individual parts:

Sample A: Comparison sample without additive.

Sample B: 300 mg. of Substance I.

Sample C: 1 g. of Substance III.

Sample D: 1 g. of Substance IV.

Sample E: 300 mg. of Substance V.

Sample F: 300 mg. of Substance VI.

Sample G: 300 mg. of Substance VII.

Sample H: 300 mg. of Substance VIII.

Sample I: as in Example 2.

Sample K: as in Example 2.

Sample L: as in Example 2.

## EXAMPLE 5

The example illustrates the comparative ineffectiveness of the substances according to the invention in a silver chloride emulsion which does not contain a color coupler. The following casting additives

5 ml. of a 1 percent aqueous solution of  $\alpha$ -phenyl-5-mercaptop-tetrazole as stabilizer,

2 g. of saponin as wetting agent, and

2 ml. of a 10 percent solution of formalin as hardener are added per kg. of a silver chloride gelatine emulsion which has a silver chloride content of 15 g. per kg. of emulsion and which has been prepared in the usual manner.

The emulsion obtained in this way is divided into five parts and the following substances are added to each part:

Sample A: Comparison sample without additive.

Sample B: 300 mg. of Substance I.

Sample C: 300 mg. of Substance II.

Sample D: 300 mg. of Substance III.

Sample E: 300 mg. of Substance VII.

This casting solution is applied onto a baryta coated paper support, exposed behind a grey step wedge and developed at 20° C. for 1 minute in a developer of the following composition:

Water—750 ml.

p-methylaminophenol—1 g.

Sodium sulfite anhydrous—13 g.

Hydroquinone—3 g.

Soda anhydrous—26 g.

Potassium bromide—1 g.

Water up to—1,000 ml.

TABLE 5

| Sample | Sensitivity | $\gamma$ | Fog  |
|--------|-------------|----------|------|
| A      | Standard    | 2.74     | 0.06 |
| B      | $\pm 0$     | 2.74     | 0.06 |
| C      | $+0.1$      | 2.75     | 0.06 |
| D      | $\pm 0$     | 2.72     | 0.06 |
| E      | $+0$        | 2.74     | 0.06 |

A difference of 3.0 corresponds to a sensitivity difference of one shutter stop.

We claim:

1. A light-sensitive photographic material with at least silver halide emulsion layer which contains a color coupler capable of forming a dye upon reaction with the oxidation product of a color-forming developer, the said silver halide emulsion layer is chemically sensitized by a water-soluble quaternization product of a  $\alpha\omega$ -bis-(thiomorpholinyl)-alkane with a bifunctional polyalkylene oxide.

2. The light-sensitive photographic material of claim 1, wherein the silver halide emulsion layer contains a chemical sensitizer of the following formula:



wherein represents

$a=2$  to 6,

$n=3$  to 300,

$y=2$  to 10, and

$x=\text{an anion.}$

3. The light-sensitive photographic material of claim 2, wherein represents  $a=2$ ,  $n=23$ ,  $y=3.4$  and  $x=\text{tosyl.}$

4. The light sensitive photographic material of claim 2, 20 wherein represents  $a=2$ ,  $n=135$ ,  $y=3.7$  and  $x=\text{tosyl.}$

5. The light-sensitive photographic material of claim 2, wherein represents  $a=2$ ,  $n=270$ ,  $y=4.8$  and  $x=\text{tosyl.}$

6. A process for the production of photographic color images by exposing and developing a photographic material 25 with at least one silver halide emulsion layer which contains a color coupler, wherein the development is performed in the presence of a water-soluble quaternization products of an  $\alpha\omega$ -bis-(thiomorpholinyl)-alkane with bifunctional polyalkylene oxide derivatives.

7. The process of claim 6, wherein the quaternization product has the following formula:



\* \* \* \* \*